

# UNITED STATES PATENT OFFICE.

ERNEST A. LE SUEUR, OF OTTAWA, ONTARIO, CANADA.

## EXPLOSIVE.

No. 923,435.

Specification of Letters Patent. Patented June 1, 1909.

Application filed November 13, 1907. Serial No. 401,944.

To all whom it may concern:

Be it known that I, ERNEST A. LE SUEUR, a citizen of the Dominion of Canada, residing at Ottawa, in the county of Carleton and Province of Ontario, Canada, have invented new and useful Improvements in Explosives, of which the following is a specification.

My invention consists of an explosive which takes advantage of the fact which I have discovered that if a mixture of suitable proportions of ground saltpeter, sulfur and a solid hydrocarbon such as paraffin wax is granulated and has then dusted over the surface of its grains a small quantity of powdered chlorate of potash, the resultant material becomes completely explosive by detonation (the original mixture being entirely insensitive to detonation) and develops much more power, cost for cost, than any explosive hitherto produced.

The following will describe the method of preparation:—Melt about 12½ lbs. of paraffin wax and add about 11 lbs. of ground sulfur, and then thoroughly mix in about 54 lbs. of ground nitrate of soda. During mixing keep the mass well loosened up with rakes or the like. Allow the mixture to cool and stiffen and then put it (preferably with brushes) through a wire screen of convenient size mesh, whereby the mass is comminuted. Then mix in about 22½ lbs. of powdered chlorate of potash, which forms a light and porous coating on the particles of the previous mixture. This makes, as stated, a powerful as well as cheap explosive, and retains its porosity sufficiently for use in bulk in rock. I may even, especially for pouring loosely into rock seams and the like, still further diminish the chlorate and yet secure good detonating properties. In such work I have even secured detonation, and the liberation of all the energy in the cheap initial mixture, with one quarter the above addition of

chlorate. No approach to such proportions can be made successful with the usual methods of mixing, and, on the other hand, to incorporate in the ordinary way sufficient chlorate to make the mixture of any service as an explosive would result in a treacherous compound which would be placed on the prohibited list.

I am aware that explosives have been compounded of nitrate of ammonia protected with fluid or semi-fluid hydrocarbons such as crude petroleum, petroleum jelly and the like, and with chlorate of potash worked into the mixture; and I am also aware that an explosive has been made with a solid hydrocarbon mixed first with a quantity of saltpeter and then with a (larger) amount of chlorate of potash, but I am not aware of any explosive ever having been prepared which anticipates my above described invention.

In the claims, saltpeter is understood to mean nitrate of soda or potash.

I claim—

1. An explosive consisting of grains of a mixture containing saltpeter, sulfur and hydrocarbonaceous material, coated with powdered chlorate of potash.

2. An explosive consisting of grains of a mixture containing saltpeter, sulfur and hydrocarbonaceous material, which latter is solid at ordinary temperatures, coated with powdered chlorate of potash.

3. An explosive consisting of grains of a mixture containing saltpeter, sulfur and wax, coated with powdered chlorate of potash.

In testimony whereof I have signed my name to this specification in the presence of two subscribing witnesses.

ERNEST A. LE SUEUR.

Witnesses:

HELEN T. LE SUEUR,  
MAUD S. LE SUEUR.